

July 20, 1926.

1,593,071

R. J. GRUENBERG

FIRE RESISTANT FIBER ROOFING TILE

Filed Nov. 24, 1923



INVENTOR.

R. J. Gruenberg.

BY  
Carlos P. Griffin  
ATTORNEY.

## UNITED STATES PATENT OFFICE.

RAOUL J. GRUENBERG, OF SAN FRANCISCO, CALIFORNIA.

## FIRE-RESISTANT FIBER ROOFING TILE.

Application filed November 24, 1923. Serial No. 676,851.

This invention relates to a fire resistant roof tile and its object is to produce a light and strong tile which will look substantially like the ordinary fired tile without its weight and with equal durability and water-proof qualities.

Another object of the invention is to produce a tile which will be initially so formed as to avoid any tendency to flatten out after it has been placed in position on the roof.

In attaining these objects a fire resistant fibrous material of the required lightness is found in rice hulls which form the base of the tile produced. These hulls are very light and contain about 18% ash which makes them burn with great difficulty.

Other objects of the invention will appear as the description proceeds.

An embodiment of the invention is shown in the accompanying drawings in which the same reference numeral is applied to the same portion throughout, but I am aware that there may be modifications thereof.

Fig. 1 is a perspective view of one form of tile,

Fig. 2 is a perspective view of another form of tile produced.

The numeral 1 indicates a half round tile which is a common form produced, while 2 indicates the convex side and 3 the concave side of an S-shaped tile which may be used instead of the shape shown in Fig. 1.

The tile consists of a mixture of asphalt, rice hulls fibrous material and mineral matter all thoroughly mixed and formed into the shapes desired.

After being formed, the tiles are subject to a pressure of several hundred pounds per square inch to properly solidify the mass, and after such pressure has been applied they are ready to be piled up to cool or to dry as the case may be, but in any event the

forming initially brings the material to the shape indicated so that when completely hardened there is no tendency for the tiles to flatten out.

The fibrous materials used may be paper fiber, asbestos fiber or mineral wool and a filling of broken stone or brick may be added, but the rice hulls and asphalt must always be in sufficient quantity to give the other materials going into the product the necessary adhesion and lightness to make an acceptable product.

The particular materials forming this product are specifically claimed in an application for patent serial number 676,850 filed of even date herewith, and are not claimed herein.

The tiles may also be formed in an ordinary clay tile machine if great pressure is applied thereto.

What I claim is as follows, but modifications may be made in carrying out the invention shown in the drawings and in the above particularly described form thereof, within the purview of the invention, as defined by the annexed claims.

I claim:

1. A roofing tile consisting of asphalt, rice hulls and fibrous materials thoroughly mixed and shaped into a tile.

2. A roofing tile consisting of a mixture of asphalt, rice hulls and mineral wool with a filling of broken stone.

3. A roofing tile consisting of a mixture of asphalt, rice hulls, fibrous material and mineral matter, moulded under heavy pressure to form a tile.

In testimony whereof I have hereunto set my hand this 14th day of November A. D., 1923.

RAOUL J. GRUENBERG.